

## UNITED STATES PATENT OFFICE

HANS RICHARD HAERTEL, OF WRENTHAM, MASSACHUSETTS, ASSIGNOR TO THOMAS H. DUMPER, TRUSTEE, OF NEWTON, MASSACHUSETTS

## RUBBERIZED ARTICLE

No Drawing.

Application filed October 23, 1928. Serial No. 314,548.

My invention relates to rubberized articles, such as raincoat material, and particularly but not exclusively to colored articles.

Heretofore it has been common practice to produce raincoat material and like goods by applying one or more layers of suitably prepared and colored rubber compound to a textile sheet by use of a calendering machine, after which the rubberized sheet is cured.

10 The constituents of the rubber compound for raincoat and like goods made according to prior methods vary widely, but commonly comprise about 35 to 60 percent rubber, about 8 percent zinc oxide, about 3 percent sulphur, 15 about 1 to 2 percent "accelerator", about 2 to 4 percent color, a small amount of anti-oxidant, and the remainder filler such as whiting, clay, and the like.

10 The zinc oxide component of the rubber compound gives tensile strength to the material; also I have found it acts to secure, in respect to the product, certain beneficial results, commonly and somewhat loosely termed that of "activating" the accelerator, 25 and, in respect to this action, to secure a satisfactory product must be used in relatively large amounts. The coloring material, commonly a lake or toner, for most colors must be used in large amounts to counteract the "dulling" effect of the zinc oxide. In common practice colors may vary in cost 30 from two to six dollars per pound, and owing to the large amounts employed constitute a considerable part of the total cost of the rubber compound. Owing to the presence of the large amount of zinc oxide in the compound prepared according to prior methods, it is impossible to secure the full effect of 35 most colors, and many colors it is impossible to use. If the amount of zinc oxide in the compounds is reduced in an attempt to improve the effect of the coloring material, the accelerator will not be effectively "activated", which will result in "blooming" and other 40 discoloration, while the product will be weakened and subject to premature decomposition.

45 By the present invention I have found that an economic saving in expensive coloring material may be effected, while at the same time

securing improved color effects and an improved product, by applying the rubber compound in at least two layers to the textile sheet or other backing prior to curing, the coloring material being confined so far as possible to the final layer, which is preferably relatively thin, while the "activator" for the accelerator in the final layer is confined so far as possible to the underlying compound.

50 For example, I have found that, largely considered, only enough zinc oxide need be retained in the final layer to give that layer its desired physical properties, and that the "activating" of the accelerator therein may be effected by including in the base layer that zinc oxide which is omitted from the final layer. The employment of a minimum of zinc oxide in the final layer materially reduces the necessary amount of color in that 55 layer, while improving the effect of such color, and renders possible the use of many colors which in the practice of prior methods it has been impossible to use, and owing to the increased effect of the color makes it in 60 most cases possible to omit the color entirely from the lower layers. The economic saving 65 in color by the improved method is very large; for example, I have found in some cases that only about 1/3 the usual percentage 70 of color need be employed in the final layer, even when the color is entirely omitted from the lower layer, and that in such cases the final layer, even when somewhat transparent, need be only about 1/3 the total thickness 75 of the rubber coating, resulting in the use of only about 1/9 the color necessary to employ in the practice of prior methods.

80 As an example of one way of practising the improved process, but without limitation 85 thereto, compound for a base layer may be prepared, by milling, consisting of:

|                                 | Per cent  |
|---------------------------------|-----------|
| Pure rubber                     | 40        |
| Zinc oxide                      | 12 95     |
| Sulphur                         | 1/2       |
| Diphenylguanidine (accelerator) | 1/2       |
| Whiting                         | remainder |

100 A layer of the above compound, about 1/32 of an inch thick, may then be applied to a

textile sheet by use of a calendering machine, and while the rubber layer is hot and tacky the surface may be wet by use of a "doctor" roll to apply thereto a film of solution consisting of a metal carbonate such as magnesium, zinc, silver, or lead carbonate, or other metal carbonate inert with respect to rubber, dissolved in ammonia water, which solution, when allowed to dry, will coat the rubber surface with a film of metal carbonate destroying its tackiness and permitting it to be rolled for further handling. As a satisfactory solution I have found practical 2 pounds magnesium carbonate dissolved in 4 gallons of 26° Baumé ammonia water.

15 A final layer of about 1/64 of an inch thick may then be applied to the material, such layer compounded by milling, and, for example, consisting of:

|                                 | Per cent  |
|---------------------------------|-----------|
| 20 Pure rubber                  | 40        |
| Zinc oxide                      | 4         |
| Sulphur                         | 1/2       |
| Diphenylguanidine (accelerator) | 1/2       |
| 25 Blue-toner (color)           | 1         |
| Whiting                         | remainder |

After the final layer is applied the rubber surface may be coated with metal carbonate as above described. It may then be varnished and cured, the curing for example consisting in subjecting the material to 270° Fahrenheit for three hours.

According to the practice of the prior method, with the same rubber content (about 35 40 percent) as in the above example, about 8 percent zinc oxide would be necessary and 2 to 3 percent color, the exact amount of color depending upon the particular color employed. It will thus be observed in the above 40 example of the practice of the improved method that, as compared to prior methods, the relatively thick base layer contains an excess of zinc oxide and no color, and that the final, relatively thin layer contains a minimum of zinc oxide and a reduced amount of color, resulting among other things, as heretofore pointed out, in a great saving of color. Further, as the base layer according to the present invention contains an excess of zinc 50 oxide, it is given an increased tensile strength, resulting in a very durable product, and especially when this layer constitutes most of the thickness of the rubber compound applied to the textile sheet. The final layer however 55 need not be thinner than the base layer as I have found that effective results may be obtained when different relative thicknesses of the two layers exist, as for example when they are of the same thickness.

60 In respect to the economic saving from the reduced amount of color, according to the prior method when 40 percent rubber at twenty cents per pound is employed, sufficient compound for covering 100 square yards of textile sheet will cost approximately

thirty-five dollars for most colors, while by the improved method the same amount of compound will cost about twenty-five dollars, thus effecting a saving of about 29 percent. With compound employing "gas-black" as 70 coloring material I have found that according to the prior method it is impossible to produce a satisfactory product, for the probable reason that gas-black, when used in amounts sufficient to give full effect of its 75 color, acts to neutralize the activating effect of the zinc oxide, but that by the improved method, owing to the reduced amount of zinc oxide therein employed and consequent reduced necessary amount of color, the full 80 color effect of this coloring material may be obtained and a satisfactory product produced.

85 Any of the various coloring materials common to the art may be employed in the practice of the invention, as for example various color-lakes and color-toners in almost any desired color and shade. The rubber content of the compound may be varied within wide 90 limits, say from 30 to 60 percent of the compound with addition of substances such as "anti-oxidants" and the like for imparting special physical or chemical properties to the compound, as desired or deemed expedient. The invention is not limited to the use of any 95 particular accelerator, and as substitutes for diphenylguanidine I may employ any of the accelerators commonly used by rubber manufacturers, as for example sulpho-carbanilide, phenylamine, urea, thiourea, mono-phenylthiourea, diphenylthiourea, mono-phenylguanidine, triphenylguanidine, other 100 amines, ureas, guanidines, and in fact any accelerator with which best results are secured by use of zinc oxide, and which will not cause undesired discoloration of the coloring material the amount of the particular 105 accelerator employed in each instance being according to its known effectiveness for the purpose and the amount of sulphur employed, the sulphur content, as will be understood by those skilled in the art, varying with the rubber content. The amount of zinc oxide may be varied to suit the desired physical 110 properties of the product, and for usual requirements 12 parts zinc oxide to 40 parts rubber in the base layer and 4 parts zinc oxide to 40 parts rubber in the final layer will give satisfactory results.

115 If desired, the tackiness of the rubber surface of the base layer may be eliminated, prior to applying the final layer, by other methods, as for example by dusting with clay, or by halogenization, or treatment with organic salt such as zinc stearate; or the material, 120 after the base layer has been applied, may be handled by winding it in the receiving roll with a superimposed textile layer to prevent adherence of the tacky rubber surface to the textile backing of the material. I have found,

however, that treatment of the rubber surface of the base layer with metal carbonates, which may be uniformly applied to give effective results in an exceedingly thin film, results in better adherence of the final layer than with prior methods, permitting the rubber surface to be embossed in an embossing press with practically no loss of material from separation of the two layers. I have also found that halogenization and treatment with organic salts decreases the elasticity of the product, decreases its durability, and when applied to the colored rubber dulls the color and makes necessary the use of additional color to overcome this dulling effect. Rolling the material with an auxiliary textile sheet to prevent sticking of the rubber surface to the textile backing, which commonly is flannel, can be done only with expenditure of a large amount of labor owing to the necessary handling, preparing and cleaning of the auxiliary layer, and, as compared to this method, I have found that by use of the improved method I can reduce the number of operators for each calendering machine from about 11 to 5 men.

From the foregoing it will be understood that it is commonly necessary to use zinc oxide with an accelerator to secure best results, the action of the zinc oxide, although it is not wholly understood, being commonly termed that of "activating" the accelerator, usually in the sense that the action of the accelerator is aided or increased by the zinc oxide. However, as the authorities differ or are in doubt as to the manner in which zinc oxide acts to secure best results with particular accelerators, in the appended claims to prevent confusion the effect of zinc oxide on the accelerator is defined as that of securing "beneficial action" of the latter, it being understood that by these words, or words of like import, it is intended to include what is commonly termed "activating" of the accelerator, where that is the beneficial result necessary with the particular accelerator employed, or the securing of any beneficial action necessary to affect best results in respect to the product as relates to the effect due to the presence of the particular accelerator employed.

It will be understood that the above description of the improved method, product, and materials employed, is given only as an example of the invention, and that wide deviations from these may be made without departing from the spirit of the invention.

**Claims:**

1. In a method of making cured colored rubber products, the improvement which comprises placing the rubber in superimposed layers, the outer layer containing color, sulphur and accelerator, and the remaining rubber containing sufficient zinc oxide effectively to secure beneficial action of the accelerator

in said outer layer during curing of the product.

2. In a method of making cured colored rubber products, the improvement which comprises placing the rubber in superimposed layers, the outer layer containing color, sulphur and accelerator, and the remaining rubber containing sulphur, accelerator and sufficient zinc oxide effectively to secure beneficial action of the accelerator in all layers

70

75

3. In a method of making cured colored rubber products, the improvement which comprises placing the rubber in superimposed layers, the outer layer containing the color, and all layers containing zinc oxide, sulphur and accelerator, the amount of zinc oxide in said outer layer being insufficient effectively to secure beneficial action of the accelerator therein, but the aggregate amount of zinc oxide present in said layers being sufficient effectively to secure beneficial action of the accelerator in all layers.

80

85

4. In a method of making cured colored rubber products, the improvement which comprises placing the rubber in superimposed layers, all of which contain sulphur, zinc oxide and accelerator, the outer layer containing color and only sufficient zinc oxide to improve its tensile strength, but the aggregate amount of zinc oxide in said layers being sufficient effectively to secure beneficial action of the accelerator in all layers.

90

95

5. That improvement in the method of producing colored rubberized material which comprises applying the rubber compound to the backing in two layers, the final layer containing coloring material and both layers containing sulphur, zinc oxide, and accelerator, the amount of zinc oxide in the final layer being insufficient effectively to secure beneficial action of the accelerator therein, but the aggregate amount of zinc oxide in both layers being sufficient effectively to secure beneficial action of the accelerator in both layers, and afterward curing the material.

100

105

6. That improvement in the method of producing colored rubberized material which comprises applying two layers of milled rubber compound to a textile sheet by use of a calendering machine, the coloring material being confined to the final layer and both layers containing sulphur, zinc oxide, and accelerator, the amount of zinc oxide in the final layer being insufficient effectively to secure beneficial action of the accelerator therein, but the aggregate amount of zinc oxide in both layers being sufficient effectively to secure beneficial action of the accelerator in both layers, and afterward curing the material.

115

120

7. That improvement in the method of producing colored rubberized material which comprises applying to a textile sheet a base layer of rubber compound containing sul-

125

130

phur, zinc oxide, and accelerator, coating the surface of said base layer with a film of metal carbonate, applying a second layer of rubber compound containing sulphur, zinc oxide, accelerator, and coloring material, and afterward curing the material, said second layer containing insufficient zinc oxide effectively to secure beneficial action of the accelerator therein, but both layers in the aggregate containing sufficient zinc oxide effectively to secure beneficial action of the accelerator in both layers.

8. That improvement in the method of producing colored rubberized material which comprises applying to a textile sheet a plurality of layers of rubber compound containing sulphur, zinc oxide, and accelerator, the final layer containing the coloring material, the amount of zinc oxide in the final layer being insufficient effectively to secure beneficial action of the accelerator therein, but the aggregate compound containing sufficient zinc oxide effectively to secure beneficial action of the accelerator in all layers.

25 9. The method of producing colored rubberized material which comprises applying to a textile sheet a plurality of layers of rubber compound containing sulphur, zinc oxide, and accelerator, the final layer being relatively thin and containing the color, the amount of zinc oxide in the final layer being insufficient effectively to secure beneficial action of the accelerator therein, but the aggregate compound containing sufficient zinc oxide effectively to secure beneficial action of the accelerator in all layers.

10. The method of producing colored rubberized material which comprises applying to a textile sheet a plurality of layers of rubber compound containing sulphur and accelerator, the final layer containing the color, and the remaining compound containing sufficient zinc oxide effectively to secure beneficial action of the accelerator in the final layer.

45 11. That improvement in the method of producing vulcanized rubberized textile sheets which comprises applying to the textile sheet two layers of rubber compound, the outer layer of which is colored, and both 50 layers containing sulphur, zinc oxide, and accelerator, the total zinc oxide present being sufficient effectively to secure beneficial action of the accelerator in both layers, but the percentage amount thereof in the inner layer being materially greater than that in the outer layer.

12. That improvement in the method of producing vulcanized rubberized textile sheets which comprises applying to the textile sheet two layers of rubber compound, the outer layer of which is relatively thin and colored, and both layers containing sulphur, zinc oxide, and accelerator, the total zinc oxide present being sufficient effectively to 65 secure beneficial action of the accelerator in

both layers, but the percentage amount thereof in the inner layer being materially greater than that in the outer layer.

13. That improvement in the method of producing vulcanized rubberized textile sheets coated, preparatory to curing, with a relatively thick base layer and a colored relatively thin finishing layer of rubber compound containing, for both layers, sulphur, zinc oxide, and accelerator, which comprises omitting from the compound of the finishing layer part of the zinc oxide necessary effectively to secure beneficial action of the accelerator therein and incorporating such part into the compound of the base layer.

70 14. Vulcanized rubberized sheet material comprising a textile sheet coated with a base of rubber compound containing a relatively large amount of zinc oxide, and a finishing layer of rubber compound containing coloring material and a relatively small amount of zinc oxide.

80 15. Vulcanized rubberized sheet material comprising a textile sheet coated with a relatively thick base of rubber compound containing a relatively large amount of zinc oxide, and a relatively thin finishing layer of rubber compound containing coloring material and a relatively small amount of zinc oxide.

85 16. Vulcanized rubberized sheet material comprising a textile sheet coated with a base of rubber compound containing a relatively large amount of zinc oxide, and a finishing layer of rubber compound containing coloring material and a relatively small amount of zinc oxide sufficient to give it material tensile strength.

90 17. Vulcanized rubberized sheet material comprising a textile sheet coated with a relatively thick base of rubber compound containing a relatively large amount of zinc oxide, and a relatively thin finishing layer of rubber compound containing coloring material and a relatively small amount of zinc oxide sufficient to give it material tensile strength.

100 18. Vulcanized rubber articles comprising a base of rubber compound containing a relatively large amount of zinc oxide, and a finishing layer of rubber compound containing coloring material and a relatively small amount of zinc oxide.

105 19. Vulcanized rubber articles comprising a relatively thick base of rubber compound containing a relatively large amount of zinc oxide, and a relatively thin finishing layer of rubber compound containing coloring material and a relatively small amount of zinc oxide.

110 20. Vulcanized rubber articles comprising a base of rubber compound containing a relatively large amount of zinc oxide, and a finishing layer of rubber compound containing coloring material and a relatively small amount of zinc oxide.

amount of zinc oxide sufficient to give it material tensile strength.

21. Vulcanized rubber articles comprising a relatively thick base of rubber compound containing a relatively large amount of zinc oxide, and a relatively thin finishing layer of rubber compound containing coloring material and a relatively small amount of zinc oxide sufficient to give it material tensile strength.

22. In testimony whereof, I have signed my name to this specification.

HANS RICHARD HAERTEL.

15

20

25

30

35

40

45

50

55

60

65